

## 1

2,734,863

## PHOSPHO-SULFURIZED HYDROCARBONS

Robert H. Jones, Irvington, N. Y., and Max W. Hill, Somerville, and Leonard E. Moody, Cranford, N. J., assignors to Esso Research and Engineering Company, a corporation of Delaware

No Drawing. Application November 1, 1951,  
Serial No. 254,442

21 Claims. (Cl. 252—32.7)

This invention relates to improved methods for preparing and treating phospho-sulfurized hydrocarbons and derivatives thereof and to improved lubricating oil compositions containing the resulting materials.

It is known to use phospho-sulfurized hydrocarbons as lubricant additives. These materials and their guanidino and reactive olefinic derivatives are stable under usual operating conditions, have beneficial detergent and antioxidant properties, and are particularly desirable for use as engine lubricants because they contain no metallic constituents and hence do not form metal-containing deposits or ash. Such additives, however, are not completely stable under storage conditions, sometimes have poor odor, and in other cases are corrosive to bearing metals and other engine parts under operating conditions.

It is the principal object of the present invention to disclose a novel method for treating the phospho-sulfurized materials with iron or copper under conditions such that improvements are obtained in the additive and in oils containing the additive. The results are unexpected since it has been conventional in the art to employ glass- or enamel-lined equipment or other ceramic-type reaction zones for the preparation of phospho-sulfurized hydrocarbons in order to avoid degradation of the product. It now has been found that treatment in the presence of these metals improves rather than degrades the material. Treatment with iron is particularly beneficial and is preferred in the present invention.

In accordance with the present invention, treatment with at least one of the metals heretofore mentioned is carried out during at least one stage of the preparation of the phospho-sulfurized hydrocarbon or the guanidino and reactive olefinic derivatives thereof. The treatment is conducted at an elevated temperature for a sufficient time and with adequate contact with the metal surface to form a stable, non-corrosive material that is substantially free of iron and copper.

The treatment is carried out at a temperature above about 300° F., preferably above 400° F. As a rule, it is preferred that the temperature not exceed about 500° to 600° F. since degradation of the product may occur at higher temperatures. The treatment will be carried out for a time sufficient to stabilize the material, the time depending upon the type of material being treated as well as the extent of metal surface present and the temperature. A time in the range of about ½ to 10 hours will generally be sufficient.

The amount of iron or copper or mixtures thereof employed during the treatment may be varied considerably. It is preferred that at least a portion of the metal be in finely divided form, such as powder, shavings, pellets, shot, steel wool and the like. The finely divided metal may be added to the material with stirring and the stirring continued during at least part of the treating period in order to insure good contact. In such cases, in the range of about 0.5 to 50% by weight, preferably about 2 to 30% by weight, based on the material being

## 2

treated will be adequate for stabilization purposes. After the treating or soaking period has been completed, the solid material is separated from the phospho-sulfurized material by filtration, such as through a diatomaceous earth or the like, or by other means.

The treatment may also be carried out in a reactor or treating vessel constructed of iron or copper or in a reactor that is lined with one of these metals. In this case, it is essential that efficient stirring or agitating devices be employed in order to obtain contact of the metal surface by the material being treated. The metal surface should be free of oxide or sulfide films or the like which generally render the metal inactive for performing the desired stabilizing function. Metal-lined treating zones may be activated by washing with a dilute mineral acid, polishing, or the like before use, water washing if necessary to remove excess acid and drying. The iron may be in the form of pure iron, cast iron, mild steel, steel alloys including small amounts of other alloying metals, and the like.

Treatment in a metal lined container is generally less preferable than treatment with a finely divided metal; in the former case it is difficult to control the extent of contact with a metal surface and deactivating films frequently formed thereon. In addition longer treating times are usually required in the case of the metal-lined reactors. A preferred procedure is to carry out the reaction or treatment in a zone lined with the desired metal and employ at the same time a smaller amount of finely divided metal than would be used in the case where the treatment is carried out in a glass- or enamel-lined reaction zone.

The metal treating step may occur at one or more stages of the preparation of the phospho-sulfurized hydrocarbon or its derivatives. For example, the phospho-sulfurization may be carried out at the conventional conditions of temperature and time of contact in the presence of metal as heretofore described, followed by filtration if necessary. The presence of the metal does not affect adversely the phospho-sulfurization step nor does the metal form a salt or other organo-metallic constituent that remains in the finished products. If desired, the phospho-sulfurization step may be conducted by conventional procedures following which the finished product is after-treated with the metallic material. The phospho-sulfurized hydrocarbon prepared by either of the above procedures may be used as such or may be further treated with guanidino or reactive olefinic compounds by procedures to be described hereinafter to produce superior ashless detergents.

In other and preferred modifications, the phospho-sulfurized hydrocarbon produced by conventional procedures is reacted with guanidino or reactive olefinic compounds in the presence of iron or copper or the guanidino and reactive olefinic derivatives may be after-treated with these metals. While the preparation should include at least one treatment with the metal, it may be desired to contact the material with the metal during two or more stages of the preparation. For example, the phospho-sulfurization step may be carried out in an iron reactor, the guanidino derivative formed, and the resulting product treated with powdered iron or copper. It will be obvious to one skilled in the art that other modifications and combinations may be employed.

The phospho-sulfurized hydrocarbon used in the present invention is one prepared by procedures well known to the art. Conveniently it is prepared by reaction of a substantially non-olefinic hydrocarbon material with a reactive sulfur- and phosphorus-containing material which is defined herein as being a sulfide of phosphorus, which may be  $P_2S_3$ ,  $P_2S_5$ ,  $P_4S_3$ , and  $P_4S_7$ , or mixtures of the elements sulfur and phosphorus or other such reactive

materials. Preferably, phosphorus pentasulfide,  $P_2S_5$ , is used. The phospho-sulfurization is generally carried out at a temperature of about 200° F. to about 600° F., and preferably from about 300° F. to about 550° F., using from about 1 to about 10, preferably about 2 to about 5, molecular proportion of the sulfide of phosphorus. The reaction is preferably carried out in a non-oxidizing atmosphere, such as an atmosphere of nitrogen. It is usually desirable to use an amount of a phosphorus- and sulfur-containing material that will give a product having at least about 1.0 weight % of both sulfur and phosphorus in chemically combined form. The reaction time is generally not critical, the time required being that to cause a practically maximum proportion of the reactive sulfur and phosphorus-containing material to react under the temperature conditions employed. A reaction time from 2 to 10 hours is generally necessary. The time should be adequate for substantially complete reaction. If desired, the reaction product may be further treated by blowing with steam, alcohol, ammonia, or the like at an elevated temperature in the range of about 200 F. to improve the odor thereof, but this further treatment is generally unnecessary since metal treatment substantially accomplishes such improvements.

A wide variety of non-olefinic hydrocarbon materials may be reacted with the phosphorus sulfide. Such hydrocarbons include paraffins, aromatics, cyclo-aliphatics, petroleum fractions, such as lubricating oil distillates, petrolatums, waxes, or condensation products of petroleum fractions, solvent extracts of petroleum fractions, and the like. Aromatic hydrocarbons such as benzene, naphthalene, anthracene, xylenes, and those having alkyl substituents and aliphatic hydrocarbons having aryl substituents may be employed. Condensation products of halogenated aliphatic hydrocarbons with an aromatic compound produced by condensation in the presence of a Friedel-Crafts type catalyst may be used. Particularly desirable, and preferred in the practice of the present invention, are essentially non-olefinic lubricant base stocks such as bright stock residuums and the like. Substantially non-olefinic hydrocarbons that have been phospho-sulfurized do not react with the metal treating agent in such manner as to form organo-metallic materials or other ash-forming constituents that remain in the finished product. It is desirable to avoid these.

The guanidino derivatives of the phospho-sulfurized hydrocarbon are prepared by neutralizing the titratable acidity of the above phospho-sulfurized reaction product (metal-treated or untreated) with guanidine or a derivative thereof. The free base guanidine and its derivatives may be used as well as basic acting salts of such bases, by which is meant salts of acids whose strength, measured on a pH scale, is less than the acidic phosphorus-sulfide hydrocarbon product. Such basic acting salts include the carbonates of guanidine and its derivatives. The products may be formed if desired by double decomposition of a salt of guanidine or guanidine derivative, such as guanidine hydrochloride or sulfate, with a metal salt of the phospho-sulfurized hydrocarbon reaction product. Although guanidine and its salts are preferred, substituted guanidines may be used.

Broadly, guanidino compounds used in the practice of the present invention may be defined by the formula



in which R, R', and R'' represent hydrogen or hydrocarbon groups containing 1 to 20 carbon atoms, e. g., straight chain alkyl groups, such as methyl, ethyl, propyl, butyl and also higher straight and branched chain alkyl groups, such as octyl, isoctyl, 2-ethylhexyl, decyl, dodecyl, tetradecyl, cetyl and stearyl radicals. R, R' and R'' may also represent cycloalkyl, arylalkyl, aryl or alkylaryl groups, as previously mentioned, for example, methylcyclohexyl, phenylethyl, phenyl, cresyl, and tert.-butyl-

phenyl groups. It will be understood that R, R' and R'' can be the same or different atoms or groups in the same molecule. However, in the case of a substituted guanidine it is most preferable to employ symmetrically tri-substituted compounds, and alkyl and cycloalkyl groups are the more preferred types of substituting groups. These include the symmetrical trialkyl, tri-naphthyl, and tri-arylalkyl guanidines. Also highly preferred classes of substituted guanidines include the monoalkyl, mononaphthyl, and monoaralkyl guanidines; unsymmetrical dialkyl dinaphthyl, and diarylalkyl guanidines. Somewhat less preferable but still useful classes are the symmetrical dialkyl, dinaphthyl, and diarylalkyl guanidines, and the mono-, di-, and triaryl guanidines. Still other substituted guanidines may be used, such as biguanide, dicyandiamide, and dicyandiamidine.

In addition to guanidine, the following specific guanidino derivatives may be used:

- 20  $\alpha$ -Methylguanidine
- $\alpha$ -Decylguanidine
- $\alpha,\alpha$ -Diisoamylguanidine
- $\alpha,\alpha$ -Dicyclohexylguanidine
- $\alpha,\alpha$ -Diphenylguanidine
- 25 Triethylguanidine
- Tribenzylguanidine.

The substantially neutralized phospho-sulfurized hydrocarbon product is prepared by reaction with a basic guanidino-compound of the above type, preferably in a non-oxidizing atmosphere, by contacting the latter with the phospho-sulfurized material as such or dissolved in a suitable solvent such as naphtha at a temperature of about 100° F. to 400° F. It is generally desired to employ at least enough of the basic compound to neutralize the titratable acidity of the phospho-sulfurized hydrocarbon product. In practice a somewhat greater amount of basic compound is generally used since the basic compound can be reacted in proportions greater than that required for neutralization of titratable acidity. When the basic compound is added in the form of a carbonate, the completion of the reaction is indicated by a cessation of carbon dioxide evolution. A water-soluble basic compound such as guanidine carbonate may be dissolved in water and then contacted with the phospho-sulfurized hydrocarbon. Metal treatment may then be carried out if desired.

The metal-treated or untreated phospho-sulfurized hydrocarbon may instead be reacted with an unsaturated hydrocarbon to form the olefinic derivative by contacting the two materials at room temperature. More preferably a somewhat elevated temperature of the order of 150°-380° F. is used with from about 0.1% to 50%, preferably about 5% to 20%, by weight of the unsaturated hydrocarbon, based on the amount of phospho-sulfurized hydrocarbon present.

The reaction is continued for a period of about one to about ten hours. The unreacted olefin is removed from the final product by distillation. However, in certain instances it may be desirable to employ an excess of the olefinic material or other unsaturated hydrocarbon products, then adding a sufficient quantity of sulfur to form a still more effective addition agent. This last step may also be made more effective by the addition of an agent commonly used in the vulcanization of rubber, such as Tuads, Captax, Tellurac, or Selenac. After-treatment with iron or copper may then be conducted, usually at a temperature above that used in forming the olefinic derivative.

The unsaturated hydrocarbon material which is reacted with the phospho-sulfurized hydrocarbon in accordance with the present invention may be any aliphatic, cyclo-aliphatic, terpenic, or aliphatic-aromatic hydrocarbon containing at least one olefinic double bond carbon-to-carbon linkage in a non-aromatic group. The materials more preferably employed include the olefins, e. g., propylene, 75 butylenes, diisobutylene, triisobutylene, the codimer of

isobutylene and n-butylene, also cracked gasoline fractions, cracked paraffin wax, viscous olefin polymers such as medium or high molecular weight polybutene, cyclopentene, cyclohexene, butadiene, pentadiene, isoprene, dipentene,  $\alpha$ -pinene,  $\beta$ -pinene, terpinolene,  $\Delta^2,4(8)$ -p-menthadiene, tyrene, and the like. Derivatives of the above described compounds containing various non-reactive substituent groups and atoms may be used to advantage, since such groups or atoms would not interfere with the reaction. Such substituted groups and atoms include nitro groups, halogen atoms, etc. Hydrocarbon materials containing from 2 to 30 carbon atoms per molecule may generally be employed. Terpenes are especially preferred.

Since the additives of the present invention are to be dissolved in mineral oils, the hydrocarbons which are reacted with sulfur- and phosphorus-containing material and the materials which are further reacted with the products thus formed will be chosen with a view to provide a product which is soluble in the oil base or which has such marginal solubility that it can be plasticized with a high molecular weight alcohol, esters, or other plasticizer.

When additives of the present invention are employed in mineral lubricating oils, they are preferably added in proportions of about 0.001 to about 20% and preferably 1.0% to about 12.0%. The proportions giving the best results will vary somewhat according to the nature of the additive and the specific purpose which the lubricant is to serve in a given case. For commercial purposes, it is convenient to prepare concentrated oil solutions in which the amount of additive in the composition ranges from about 20% to 50% or higher by weight, and to transport and store them in such form. In preparing a lubricating oil composition for use as a crankcase lubricant, the additive concentrate is merely blended with the base oil in the required amount.

Below are given detailed description of preparations of examples of lubricating oil additives described above as well as tests in which an oil containing the additives was used as the lubricant. It is to be understood that these examples are given as illustrations of the present invention and are not to be construed as limiting the scope thereof in any way.

*Example I.—Preparation of P<sub>2</sub>S<sub>5</sub> treated bright stocks*

Several pilot plant preparations of P<sub>2</sub>S<sub>5</sub>-treated bright stock (a solvent extracted, dewaxed, deasphalted bright stock from Mid-Continent crude) were carried out by treating the bright stock with 10% by weight of P<sub>2</sub>S<sub>5</sub> for 8–10 hours at 400° F. When the reaction was carried out in an iron (mild steel) reactor, the product was considerably more stable, as regards both the tendency to form oil-insoluble precipitates and the tendency to evolve H<sub>2</sub>S, than products obtained from the same reaction in enamel or glass reactors. This is shown by the data in the table below. It should be noted that the phosphorus contents of the products prepared in glass and iron were essentially identical but the sulfur content of the material prepared in iron was significantly lower.

PROPERTIES OF P<sub>2</sub>S<sub>5</sub>-TREATED BRIGHT STOCKS

| Product Analysis                                                          | Reactor Material |                        |
|---------------------------------------------------------------------------|------------------|------------------------|
|                                                                           | Iron             | Enamel or Glass        |
| Phosphorus, wt. percent.....                                              | 1.54.....        | 1.8-2.0.....           |
| Sulfur, wt. percent.....                                                  | 1.52.....        | 3.7-4.7.....           |
| Iron, wt. percent.....                                                    | 0.007.....       |                        |
| Storage stability after 1 month at room temperature.                      | Clear.....       | Solid Precipitate..... |
| Hydrogen sulfide stability <sup>1</sup> Pb(Ac) <sub>2</sub> rating after: |                  |                        |
| 24 hours at room temperature.....                                         | 0.....           | 10.....                |
| 10 days at room temperature.....                                          | 4.....           |                        |

<sup>1</sup> Rated by using filter paper saturated with lead acetate (Pb(Ac)<sub>2</sub>) for 5 minutes exposure; no stain is 0 and jet black is 10.

Blends containing 6.0 wt. per cent of the above reaction products in a solvent extract Mid-Continent base oil having a viscosity of 120 S. U. S. at 210° F. were subjected to copper, silver and bronze corrosion tests and in each case it will be noted that the material prepared in iron was less corrosive than the corresponding products prepared in enamel or glass.

A. *Copper corrosion*.—The test procedure was a modification of the CRC method, L-16-445, for determining the copper staining tendencies of oils, the method as modified comprising immersing a polished metallic copper strip in the oil to be tested for a period of three hours at 210° F. and noting the extent of the staining. Ratings are given on a scale of from 1 to 10 which denotes discoloration ranging from no stain to a black surface film.

B. *Silver corrosion*.—This test involves measuring the weight change and observing the discoloration of a sterling silver strip immersed in 50 cc. of the test oil for 17 hours at 325° F. The stain is rated from 0 for no discoloration to 8 for complete sulfide film. Weight changes above 1.5–2.0 mgs. are considered excessive and discolorations rating above 4 are normally considered failing although the actual limits will depend on the application for which the lubricant is designed.

C. *Bronze corrosion*.—This test involved exposing a section of a bronze exhaust valve guide (attached to the end of an electrically driven stirrer) to approximately 300 cc. of the lubricating oil at 500° F. for 3 successive 4 hour periods. At the end of each period the guide section was removed, cleaned, and the weight loss determined. The total loss for the 12 hour test was calculated. Comparative data for the product prepared in the iron reactor and in enamel or glass reactors are shown in the following table:

35

CORROSION DATA FOR BLENDS OF P<sub>2</sub>S<sub>5</sub>-BRIGHT STOCKS

| P <sub>2</sub> S <sub>5</sub> treated Bright Stocks<br>Prepared in — | Copper<br>Corrosion | Silver Corrosion         |          | Bronze<br>Corrosion |
|----------------------------------------------------------------------|---------------------|--------------------------|----------|---------------------|
|                                                                      |                     | Weight<br>Change,<br>mg. | Color    |                     |
| Iron.....                                                            | 2.....              | 0.1.....                 | 4.....   | 39.....             |
| Enamel or Glass.....                                                 | 8.....              | 1.3-1.9.....             | 6-7..... | 94.....             |

*Example II.—Guanidine salts of P<sub>2</sub>S<sub>5</sub>-treated bright stocks*

Guanidine salts of the P<sub>2</sub>S<sub>5</sub>-treated bright stocks described in Example I were prepared by neutralizing the P<sub>2</sub>S<sub>5</sub>-bright stock reaction product with 10% by weight of guanidine carbonate. This was accomplished by adding 10% by weight guanidine carbonate as a 30% aqueous solution, and stripping out the water by heating the mixture in an open container using Na stripping. The temperature was gradually raised until all the water was removed, the final temperature being approximately 350° F. at which point the product was filtered. A comparison of the materials made by neutralizing in glass equipment the products prepared in Example I is given in the following table. In this case blends of 6 wt. per cent of the guanidine salts in a solvent extracted Mid-Continent base stock having a viscosity of 120 Saybolt seconds at 210° F. were subjected to the following bronze corrosion test at 650° F. Quarter sections of bronze exhaust valve guides were exposed to 50 cc. of oil (containing the additive under test) for 17 hours at 650° F. At the end of the test the sulfide film was removed by washing the strips with cyanide solution, and the weight loss per gram of section determined. It will be noted that the guanidine salt of the P<sub>2</sub>S<sub>5</sub>-treated bright stock, where the bright stock phospho-sulfurization was carried out in iron, was much less corrosive than the corresponding product made in glass or enamel.

7  
PROPERTIES OF GUANIDINE SALT OF P<sub>2</sub>S<sub>5</sub>-TREATED BRIGHT STOCKS

|                                                                                                      |      | Reactor Material |  |
|------------------------------------------------------------------------------------------------------|------|------------------|--|
|                                                                                                      | Iron | Glass and Enamel |  |
| Analysis:                                                                                            |      |                  |  |
| Percent Phosphorus.....                                                                              | 1.47 | 1.4-2.3          |  |
| Percent Sulfur.....                                                                                  | 1.68 | 1.9-2.6          |  |
| Percent Nitrogen.....                                                                                | 3.51 | 3.4-3.8          |  |
| Bronze Corrosion, 6 wt. percent, Blends, 17 Hours at 650° F., Weight Loss, mg./g. <sup>1</sup> ..... | 1.56 | 1.89             |  |

<sup>1</sup> Averages of at least 2 determinations.

Example III.—Preparation of guanidine salt of P<sub>2</sub>S<sub>5</sub>-treated bright stock totally in iron 15

In the example above only the P<sub>2</sub>S<sub>5</sub> treatment was carried out in an iron reactor. In the present example, the total reaction including the neutralization was carried out in iron. 1000 grams of a solvent extracted Mid-Continent bright stock of approximately 150 Saybolt seconds viscosity at 210° F. was charged to an ordinary black iron (cast iron) pot sitting on a hot plate. The bright stock was stirred and also blown with N<sub>2</sub> and the temperature raised to 300° F. in one-half hour. At that point 300 grams of P<sub>2</sub>S<sub>5</sub> were added and the temperature was raised to 450° F. The product was soaked at 450° F. for five hours and then filtered using "Hy-flo" filter aid while hot.

To 500 grams of the filtrate 50 grams of guanidine carbonate dissolved in 100 grams of H<sub>2</sub>O was added at about 160° F. The temperature was gradually raised to 320-340° F. and held at that point for two to three hours in order to remove all traces of moisture. It was again filtered through Hy-flo. Bronze corrosion data were obtained for a 6.0 wt. per cent blend of this product in the same base oil and by the same test as was used in Example II. The corrosion characteristics of the product were essentially equivalent or possibly slightly better than those of the product in Example II where only the bright stock was P<sub>2</sub>S<sub>5</sub>-treated in iron. A comparison is shown below:

| P <sub>2</sub> S <sub>5</sub> Treatment | Neutralization | Bronze Corrosion 17 Hours at 650° F., mg./g. | Remarks                         |
|-----------------------------------------|----------------|----------------------------------------------|---------------------------------|
| Iron.....                               | Iron.....      | 1.51                                         |                                 |
| Do.....                                 | Glass.....     | 1.56                                         | See Example II for preparation. |

Example IV.—Treatment with iron powder

A. Preparation of the P<sub>2</sub>S<sub>5</sub>-treated bright stock.—150 pounds of phenol extracted Mid-Continent bright stock was charged to a glass-lined reactor and heated to 250-275° F. with stirring and nitrogen blowing. 15 pounds of P<sub>2</sub>S<sub>5</sub> was added and the mixture heated to 400° F. over a period of 3½ hours. The reaction mixture was soaked at 400° F. for an additional 8 hours. The final product contained 1.91% phosphorus, 3.89% sulfur and had a neutralization number of 24.1.

B. Treatment of the bright-stock P<sub>2</sub>S<sub>5</sub> product with iron.—200 grams of the product prepared in A above were stirred in a glass reactor with 20 grams (10% by weight) of powdered iron. A stream of nitrogen was blown continually through the reacting materials, and after three hours at 425° F. the product was filtered. 150 grams of the final product were converted to the guanidine salt by the addition of 15 grams (10% by weight) guanidine carbonate dissolved in 30 grams of water. The mixture was slowly heated to 320° F. and held there for one hour before it was filtered. All of the reactions were carried out in glass.

The P<sub>2</sub>S<sub>5</sub>-bright stock prepared in A above was also converted to the guanidine salt, however no iron treatment was used. In this case 130 pounds of the bright stock was treated with 13 pounds of guanidine carbonate 70

in 10 pounds of water and the addition was made at 135° F. The reaction mixture was heated to 320° F. over an eight hour period and held at 320° F. for two hours before filtering.

5 200 grams of this product were then treated with 20 grams (10 wt. percent) of powdered iron for three hours at 425° F. under a nitrogen atmosphere. A comparison of the bronze corrosion characteristics of these three final products is given in the following table. All of the data being for 6 wt. percent blends of the guanidine salts in a solvent extracted Mid-Continent base oil of 100 Saybolt viscosity at 210° F. The bronze corrosion test used is that described in Example II.

| 20 | 6 Wt. Percent Blends of —                                                       | Bronze Corrosion 17 Hours at 650° F., Wt. Loss, mg./g.                       |
|----|---------------------------------------------------------------------------------|------------------------------------------------------------------------------|
|    |                                                                                 | Guanidine Salt of Untreated P <sub>2</sub> S <sub>5</sub> -Bright Stock..... |
|    | Guanidine Salt of Iron Treated P <sub>2</sub> S <sub>5</sub> -Bright Stock..... | 1.27                                                                         |
|    | Iron Treated Guanidine Salt of P <sub>2</sub> S <sub>5</sub> -Bright Stock..... | 1.62                                                                         |

Example V.—Treatment of the guanidine salt of P<sub>2</sub>S<sub>5</sub>-bright stock with metallic copper

25 30 200 grams of the guanidine salt of P<sub>2</sub>S<sub>5</sub>-treated bright stock prepared in Example IV were treated with 25 grams (12.5% by weight) of metallic copper flakes added portionwise over a two-hour period at 500° F. The product was then filtered and the effect of the copper treatment on high temperature bronze corrosion was measured for a 6 wt. percent blend. The results are shown below:

| 35 | 6 Wt. Percent Blend                                                               | Bronze Corrosion 17 Hours at 650° F., Wt. Loss, mg./g.             |
|----|-----------------------------------------------------------------------------------|--------------------------------------------------------------------|
|    |                                                                                   | Guanidine Salt of P <sub>2</sub> S <sub>5</sub> -Bright Stock..... |
|    | Copper-treated Guanidine Salt of P <sub>2</sub> S <sub>5</sub> -Bright Stock..... | 1.42                                                               |

40 Example VI.—Treatment of P<sub>2</sub>S<sub>5</sub>-treated bright stock with copper

A. Preparation of the P<sub>2</sub>S<sub>5</sub>-treated bright stock.—146.5 pounds of an acid-treated, clay-contracted, deasphalted, dewaxed bright stock from Mid-Continent crude was reacted with 31.5 pounds (21%) P<sub>2</sub>S<sub>5</sub> in a glass-lined reactor. The materials were heated to 400° F. over a two-hour period and the reaction was maintained at this temperature for 10 hours after which it was filtered through "Hy-flo." The final product contained approximately 3% phosphorus and 6% sulfur.

B. Copper treatment.—500 grams of the P<sub>2</sub>S<sub>5</sub>-treated bright stock were stirred in the presence of finely divided metallic copper at about 400° F. A total of 80 grams (16% by weight copper) was added portion-wise over the three-hour period, after which the product was filtered through "Hy-flo." Blends (2.5 wt. percent) of the P<sub>2</sub>S<sub>5</sub>-treated bright stock and of the copper-treated P<sub>2</sub>S<sub>5</sub>-treated bright stock in an SAE 30 grade solvent extracted, Mid-Continent base stock were evaluated for H<sub>2</sub>S evolution and silver corrosion. The blends also contained 2.5 wt. percent of a 30% oil concentrate of calcium petroleum sulfonate. The data summarized in the following table indicate that the copper treatment made a marked improvement in both H<sub>2</sub>S evolution and in corrosivity toward silver.

| Wt. percent blends in a Solvent Extracted Mid-Continent SAE-30 Grade Lubricating Oil | H <sub>2</sub> S Stability, 7 Days at 100° F., Pb (Ac) <sub>2</sub> Rating | Silver Corrosion |       |
|--------------------------------------------------------------------------------------|----------------------------------------------------------------------------|------------------|-------|
|                                                                                      |                                                                            | Wt. Change, Mg.  | Color |
| 2.5% Untreated P <sub>2</sub> S <sub>5</sub> -Bright Stock.....                      | 10                                                                         | 2.2              | 7     |
| 2.5% Calcium Sulfonate Concentrate.....                                              |                                                                            |                  |       |
| 2.5% Copper-Treated P <sub>2</sub> S <sub>5</sub> -Bright Stock.....                 | 0                                                                          | 0.8              | 3     |
| 2.5% Calcium Sulfonate Concentrate.....                                              |                                                                            |                  |       |

*Example VII.—Iron treatment of diisobutylene-P<sub>2</sub>S<sub>5</sub>-treated bright stock*

1000 grams of a P<sub>2</sub>S<sub>5</sub>-treated bright stock made with 10% P<sub>2</sub>S<sub>5</sub> under the conditions given in Example IV were treated with 150 grams of close-cut diisobutylene at 300° F. for three hours. At the end of that time the untreated diisobutylene was stripped out. All of the reactions were carried out in glass.

The diisobutylene-P<sub>2</sub>S<sub>5</sub>-bright stock reaction product was then treated with 20% (by weight) of finely divided metallic iron at 400° F. for three hours, after which it was filtered. These materials were evaluated for hydrogen sulfide stability, and for copper and silver corrosivity as 2.5 wt. percent blends in an SAE-30 grade solvent extracted Mid-Continent lubricating oil base stock containing 2.5 wt. percent of an oil concentrate of a calcium petroleum sulfonate.

| Additive                                                                   | H <sub>2</sub> S Stability 1 Day at Room Temperature Pb (Ac) <sub>2</sub> Rating | Silver Corrosion |       | Copper Corrosion |
|----------------------------------------------------------------------------|----------------------------------------------------------------------------------|------------------|-------|------------------|
|                                                                            |                                                                                  | Wt. Change, Mg.  | Color |                  |
| 2.5% Diisobutylene-P <sub>2</sub> S <sub>5</sub> Bright Stock              | 4                                                                                | 1.5              | 7     | 8                |
| 2.5% Calcium Sulfonate Concentrate                                         |                                                                                  |                  |       |                  |
| 2.5% Iron-Treated Diisobutylene-P <sub>2</sub> S <sub>5</sub> Bright Stock | 0                                                                                | 0.3              | 4     | 2                |
| 2.5% Calcium Sulfonate Concentrate                                         |                                                                                  |                  |       | 30               |

It will be noted that in all cases the iron treatment markedly improved the material.

*Example VIII.—Aviation C. F. R. engine evaluation*

A sample of P<sub>2</sub>S<sub>5</sub>-treated bright stock prepared in an iron reactor (Example I) was evaluated at 6.0 wt. percent in a 120 grade aviation oil in an aviation C. F. R. engine test. The results of this test show that the blend gave considerably less deposits than the base stock as illustrated in the data in the table below. The test consisted of 50 hours of operation at 1800 R. P. M. and 4 brake horsepower. The oils were rated on a demerit system where a perfectly clean surface is given a rating of zero and 10 is equivalent to the worst condition that could be expected. In the test with the base aviation oil the deposits in the critical ring zone area were very heavy (6.4 demerit) and the addition of the 6.0% P<sub>2</sub>S<sub>5</sub>-treated bright stock from the iron reactor resulted in a marked improvement (2.0 demerit). Similarly improved results were obtained when using the guanidine salt of a P<sub>2</sub>S<sub>5</sub>-treated bright stock prepared from the P<sub>2</sub>S<sub>5</sub>-treated material made in iron. These data are shown in the following table:

| 6 Wt. Percent Blends in Aviation Oil                                                   | Ring Zone Demerit |
|----------------------------------------------------------------------------------------|-------------------|
| None                                                                                   | 6.4               |
| P <sub>2</sub> S <sub>5</sub> -Treated Bright Stock prepared in Iron                   | 2.0               |
| Guanidine Salt of P <sub>2</sub> S <sub>5</sub> -Treated Bright Stock prepared in Iron | 2.9               |

The products of the present invention are particularly useful as ashless detergents in aviation engine lubricating oils and the like. They may be employed in ordinary hydrocarbon lubricating oils, in "heavy duty" type of lubricants along with other additives of the conventional types, and with various synthetic lubricants such as those prepared by polymerization of olefins, by the reaction of oxides of carbon with hydrogen, or by other means. The conventional synthetic oils of the ester, polyester and polyether types may also be used alone or in combination with mineral lubricants as base oils. The lubricating oils may vary considerably in viscosity and other properties, de-

pending on the use for which they are desired, but they usually range from about 35 to 150 viscosity (Saybolt) at 210° F.

Other agents such as pour depressors, organometallic compounds, sludge dispersers, viscosity index improvers, anti-oxidants and the like may be used along with the additives of the present invention in compounding the lubricants. In addition to being employed in lubricants, the additives of the present invention may also be used in motor fuels, hydraulic fluids, cutting oils, turbine oils, fuel oils, transformer oils, and in other petroleum products as anti-oxidants or detergents. They may also be used in gear lubricants and greases.

What is claimed is:

- 15 1. In the process of forming a product selected from the class consisting of phospho-sulfurized, non-olefinic hydrocarbon materials and the guanidino and reactive olefinic derivatives thereof, said materials containing at least 1.0 weight percent of both phosphorus and sulfur in chemically combined form; the improvement which comprises including during at least one stage of said process a contacting with a metal selected from the class consisting of iron and copper at an elevated temperature.
- 20 2. A process as in claim 1 wherein said contacting is carried out during the phospho-sulfurization of an essentially non-olefinic hydrocarbon material with a phosphorus sulfide.
- 25 3. A process as in claim 1 wherein said contacting is carried out on said phospho-sulfurized hydrocarbon.
- 30 4. A process as in claim 1 wherein said contacting is carried out on said derivatives of said phospho-sulfurized hydrocarbon.
- 35 5. A process as in claim 1 wherein said phospho-sulfurized hydrocarbon is contacted with said metal and said derivatives are formed from the contacted product.
- 40 6. A process as in claim 1 wherein said contacting with said metal is carried out at a temperature above about 300° F.
- 45 7. A process as in claim 1 wherein said contacting is carried out with from 1 to 50 weight per cent of iron in finely divided form and the contacted material is filtered to remove solid matter.
- 50 8. In the process of forming a product selected from the class consisting of the reaction products of a lubricating oil base stock with a phosphorus sulfide and the guanidino and reactive olefinic derivatives thereof, said product including at least 1.0 weight per cent of both phosphorus and sulfur in chemically combined form and being unstable and corrosive in character, the improvement which comprises including during at least one stage of said process a contacting with a metal selected from the class consisting of iron and copper at a temperature in the range of about 300°-500° F. and removing solids therefrom, whereby a substantially stable and non-corrosive product is formed.
- 55 9. A process as in claim 8 wherein said phospho-sulfurization is carried out in the presence of said metal.
- 60 10. A process as in claim 8 wherein said phospho-sulfurized product is contacted with said metal.
- 65 11. A process as in claim 8 wherein said derivatives are contacted with said metal.
- 70 12. A hydrocarbon oil composition containing a detergent quantity of a product selected from the class consisting of a phospho-sulfurized substantially non-olefinic hydrocarbon materials and the guanidino and reactive olefinic derivatives thereof, said materials containing at least 1.0 weight per cent of both phosphorus and sulfur in chemically combined form; which product has been contacted during at least one stage of the preparation thereof with a metal selected from the class consisting of iron and copper at elevated temperatures and for an extended period of time, adequate to produce a substantially odorless, non-corrosive product.
- 75 13. A composition as in claim 12 in which said non-

olefinic hydrocarbon is a lubricating oil base stock.

14. A composition as in claim 13 in which said non-olefinic hydrocarbon is a bright stock obtained from a conventionally refined petroleum residuum.

15. A composition as in claim 12 wherein said guanidino derivative is prepared by treatment with guanidine carbonate.

16. A composition as in claim 12 wherein said reactive olefinic derivative is prepared by treatment with diisobutylene.

17. A composition as in claim 12 in which said phospho-sulfurized hydrocarbon is prepared by treatment with  $P_2S_5$ .

18. A composition as in claim 12 which includes from about 0.001 to 20 weight per cent of said product.

19. A concentrate comprising essentially a lubricating oil and above about 20% of the product of claim 8.

20. In the process of forming a product selected from the class consisting of reaction products of a substantially non-olefinic hydrocarbon material selected from the group consisting of paraffins, aromatics, cyclo-aliphatics and petroleum fractions with a phosphorus sulfide and the guanidino and olefinic derivatives thereof, said product including at least 1.0 wt. per cent of both phosphorus and sulfur in chemically combined form and being unstable and corrosive in character, the improvement which comprises contacting at least a portion of said reaction

product during at least one stage of said process with a metal selected from the class consisting of iron and copper at a temperature in the range of about 300° to 500° F., whereby a substantially stable and non-corrosive product is formed.

21. In the process of forming a reaction product of a solvent extracted bright stock with phosphorus pentasulfide at a temperature of about 200° to 600° F. in a non-oxidizing atmosphere, said product having at least about 1.0 wt. per cent of both sulfur and phosphorus in chemically combined form, the improvement which comprises contacting at least a portion of said reaction product during at least one stage of said process with a metal selected from the group consisting of iron and copper at a temperature in the range of about 300° to 500° F. for about 0.5 to 10 hours.

References Cited in the file of this patent

UNITED STATES PATENTS

|    |           |               |       |               |
|----|-----------|---------------|-------|---------------|
| 20 | 2,206,151 | Bennett       | ----- | July 2, 1940  |
|    | 2,315,529 | Kelso         | ----- | Apr. 6, 1943  |
|    | 2,379,312 | May           | ----- | June 26, 1945 |
|    | 2,381,907 | Hughes et al. | ----- | Aug. 14, 1945 |
| 25 | 2,424,402 | Loane et al.  | ----- | July 22, 1947 |
|    | 2,443,823 | Holt          | ----- | June 22, 1948 |
|    | 2,460,041 | Sparks et al. | ----- | Jan. 25, 1949 |
|    | 2,560,543 | Bartleson     | ----- | July 17, 1951 |